# EUROPEAN PATENT SPECIFICATION

(11) **EP 0 043 680 B1**
(45) Date of publication and mention of the grant of the patent: **05.12.1984**
(21) Application number: 81302888.3
(22) Date of filing: 26.06.1981
(51) Int. Cl.: C23G 1/20, C23G 1/18

(54) **Process for removing contaminants from a tin surface**
Verfahren zur Entfernung von Verunreinigungen von einer Zinnoberfläche
Procédé d'élimination d'impuretés d'une surface en étain

(30) Priority: 27.06.1980 US 163566
(43) Date of publication of application: 13.01.1982
(73) Proprietor: AMCHEM PRODUCTS, INC., Ambler Pennsylvania 19002 (US)
(72) Inventor: McCready, Newton Willoughby, Newton Square Pennsylvania 19073 (US)
(74) Representative: Sanderson, Laurence Andrew

## Description

This invention relates to a process employing an aqueous alkaline solution for cleaning tin surfaces.

The invention is particularly concerned to provide a corrosion inhibitor for use in the aqueous alkaline cleaning solution which will deter or inhibit etching of the tin surface. Although the invention is applicable to the removal of contaminants from all kinds of tin surface, it will here be described in connection primarily with the cleaning of tin-plated surfaces, such as tin cans, which have been soiled with organic lubricants of the kind that are applied to the tin surface as drawing aids during cold-forming operations.

Cleaning is an essential preliminary to many surface-finishing operations. It is for example normally necessary to clean any metal surface prior to corrosion-preventive treatments, and prior to the application of organic finishes to the surface; and cleaning is especially important in the case of metal surfaces to which organic materials have been recently applied as an aid to cold-forming. Such organic lubricating materials must be removed in order to make the metal surface suitably receptive to an organic or inorganic finish.

A typical and important example of a situation where preliminary cleaning is needed can be found in the manufacture of two-piece, tin-plated, so-called "drawn-and-ironed" cans. Circular blanks of tin-plated steel (which, due to the high cost of tin, generally have only a thin layer of tin plating) are first cupped and then passed through several drawing dies, so as thus to "iron" the cup-in order thus to form a unitary side-wall and can-bottom structure. Any can produced by this process will normally have a fairly characteristics shape, i.e. it will be a thin-walled, thick-bottomed container having a generally uniform wall thickness; and such cans will be referred to herein as "DI" (drawn-and-ironed) cans.

The forming operations carried out during the manufacture of DI cans are normally assisted, and indeed the dies and the metallic surface are protected, by the application of lubricants to the tin-plate surface prior to or during the forming operation. The lubricants which are thus applied to the tin surface usually consists of various types of mineral and vegetable oils and heavy metal soaps; and they must be removed if it is desired to have a clean surface in order to assure adhesion of a subsequently applied sanitary lacquer and/or decorative varnish.

One problem with Di tin-plated containers, which can be serious, is that the drawing operation stretches the tin-plate surface, thereby exposing some of the underlying metal. The underlying metal may very probably be a ferrous metal, such as iron or one of many iron alloys or of a wide variety of steels; and its exposure may easily lead to corrosion. An effective cleaner for tin-plate is one which indeed will provide a water-break-free surface on the tin (a water-break-free surface is one which is sufficiently freed from lubricants, soil, and other contaminants so that it will maintain a continuous film of water) but which will do so without unduly etching the tin and without promoting corrosion of the underlying metal.

Etching of the tin surface results from chemical attack of the cleaning solution thereon and results in a roughened and dull surface. Inevitably etching also removes some of the corrosion-protective layer of tin from the underlying metal surface, thereby diminishing the anti-corrosion qualities of the tinned surface, and aggravating any corrosion problems arising from exposure of the underlying metal. In the case of say a beverage can, where a smooth, shiny appearance is wanted and maximum safety of the contents is necessary, it is clear that etching and/or corrosion will be highly undesirable.

Etching and corrosion can be an especially severe problem with conventional cleaners for tin-plate when during the cleaning operation line-stoppage can expose some of the cleaned cans to the cleaner for excessive periods, which can lead to etching and corrosion of the underlying metal surface (no matter whether exposed by stretching or by etching) so severe as to render the cans quite unacceptable for use. Apart from appearance, any corrosion and blemishes on the surface will adversely affect the adhesion of any chemical conversion coating or sanitary lacquer coating that may thereafter be applied to it.

The cleaners which have been found to be most suitable for producing the desired water-break-free surface on the tin are alkaline cleaners, such as aqueous solutions of alkali metal salts of silicates, phosphate, carbonates and borates- but these all have the undesirable tendency to etch the surface. Efforts have therefore already been made to discover additives which will help to inhibit etching of the tin surface under the alkaline conditions employed.

Broadly-speaking it is a fair generalization to say that the inhibited alkaline cleaning solutions hitherto suggested have mostly required the use of long periods (for instance up to 15 minutes) and/or relatively high temperatures (at least 140°F [60°C] and often above 150°F [about 65°C]) to achieve satisfactory cleaning. In many instances the suggested inhibitors give rise to waste-disposal and other problems arising from their toxicity or other characteristics.

United States Patent No. 4,094,701 discloses a process for cleaning a tin surface, without substantially etching it, using an aqueous alkaline solution containing an alkaline component as well as one or more surfactants and, serving as inhibitor, an organic tannin. This solution is sprayed on to the object to be cleaned at elevated temperature for about one to about two minutes. The pH of the cleaner is at least 9, and because higher pH values tend gradually to inactivate the tannin it is preferably between 10 and 13, and most preferably between 10 and 10.5. When in the preferred pH range of say from 9 to 10.5 this cleaner is to be employed at temperatures of 140°F (60°C) and upwards. Thus, while it is true that this United States Patent No. 4,094,701 does disclose a cleaning solution that can be used for cleaning tin. surfaces, without etching, at temperatures below boiling in periods of less than two minutes, nevertheless the use of temperatures in excess of 140°F (60°C) is still economically disadvantageous. Moreover the recommended alkaline components include alkali metal borates and phosphates, both of which may give rise to environmental problems and, hence, plant-effluent treatment problems.

There is thus today still an unfulfilled need for an effective economic and ecologically-acceptable cleaning solution and process which may be used upon tin articles operating at temperatures lower than those previously found to be effective so as to produce a water-break-free surface thereon without etching the tin, no matter whether applied for the necessary minimum periods of about one minute or less or whether by line-stoppage or other accident applied for much longer periods of time than had been intended-without the use of components currently regarded as environmentally objectionable.

We have now found that this need can be largely or even wholly fulfilled by means of the cieaning solutions and processes hereinafter described.

Accordingly, the invention provides a process for removing lubricants or other soiling contaminants from a tin surface without visibly etching it, in which the surface is brought into contact for a sufficient time at the chosen temperature with an aqueous alkaline cleaning solution having a pH in the range of from 11 to 13 and containing effective amounts of an alkaline component and of an inhibitor, characterized in that the inhibitor is or includes onr or more substituted or unsubstituted quinones and/or substituted or unsubstituted dihydroxybenzenes, the or each substituent on the quinone or dihydroxybenzene being hydroxy, halo, alkyl, alkoxy, nitro or cyano.

The term "tin" as used herein refers not merely to pure tin metal but also to alloys where in tin predominates; and the term "tin surface" refers to the surface of not only articles made of tin but also those plated with tin.

It will of course be understood that by an -."effective amount" of the alkaline component we mean such a concentration as will substantially remove the lubricants or other soiling contaminants, leaving a water-break-free tin surface. Similarly by an "effective amount" of the inhibitor we mean such a concentration as is able substantially to inhibit etching of the tin surface.

The substituted or unsubstituted dihydroxybenzenes are otherwise substituted or unsubstituted benzenes which bear at least two hydroxy substituents, in ortho-, meta- or para- positions, and perhaps more than two such hydroxy substitutents arranged either symmetrically or asymmetrically.

Exemplary quinones and substituted quinones useful as inhibitors in this invention include the substituted and unsubstituted quinones according to general formulae II and III below: in which R_{1'} R,, R₃ and R₄ are the same or different and each represents a hydrogen atom or an alkyl, alkoxy, hydroxy, halo, nitro or cyano group.

Exemplary substituted or unsubstituted polyhydroxybenzene inhibitors, of particular interest for. use in this invention, include for instance catechol (ortho-dihydroxybenzene) and/or resorcinol (meta-dihydroxybenzene) and/or hydroquinone (1,4-dihydro-benzoquinone or para-dihydroxybenzene) and/or hydroxy-hydroquinone (1,2,4-trihydroxybenzene) and/or 1,3,5-trihydroxybenzene and/or 1,2,4,5-tetrahydroxybenzene.

Preferred inhibitors for use in this invention include 1,2,3-benzene-triol and dihydroxybenzenes as well as quinones, such as 1,4-benzenediol and 1,4-benzoquinone.

The inhibitor must naturally be added in an amount effective to inhibit etching of the tin surface. Generally, the necessary minimum concentration of the inhibitor will increase with the concentration of the alkaline component. Moreover, since "soft" water tends to be more corrosive than "hard" water (as will be further discussed below) generally the necessary minimum concentration of inhibitor will tend to be greater when the cleaning solutions are made-up with soft water than when they are made-up with hard water. The concentration of inhibitor in the solution will advantageously be at least about 0.02 g/I; and it will preferably be in the range of from about 0.02 g/I to about 0.06 g/I. There is no objection to the use of concentrations greater than 0.06 g/I, but generally the resultant increase in cost is not repaid by a greater inhibition of etching.

The addition of a polyelectrolyte to the cleaning solutions used in the invention has been found to be beneficial since then the solution may be employed effectively irrespective of the hardness of the water used to make-up the solution.

Hardness is a characteristic of water, generally accepted to represent the total concentration of calcium and magnesium ions-although other polyvalent cations, seldom present in more than trace amounts, may sometimes also contribute to hardness. The determination of hardness can be carried out by titration, as described in "Standard Methods of Test for Hardness in Water", Designation D 1126-67 (Reapproved 1974) published by the American Society for Testing Materials. Hardness may conveniently be expressed in parts per million (ppm) of calcium carbonate equivalent; the higher the value, the greater being the hardness. Usually water having a hardness of less than about 100 ppm will be regarded as "soft", whereas with a hardness about 100 ppm it will be regarded as "hard". Water-hardness can vary greatly from place to place. In some coastal regions of the United States the hardness may be only about 50 ppm to about 100 ppm, but it may increase to about 300 ppm where the water runs somewhere through limestone deposits, and in some areas of the Midwest of the United States the hardness may be as much as from about 400 ppm to about 500 ppm.

When the water used to make-up the alkaline aqueous solutions used in this invention is rather hard then, unless indeed polyelectrolytes are present, there is a tendency to experience precipitation of the calcium and magnesium ions that cause water hardness. The greater the hardness of the water the greater usually will be the degree of precipitation. Any such precipitation is potentially a problem, since it may result in sediment which is liable, for example, to clog spray nozzles when spraying is the chosen method of application. The use of softer water is moreover not an altogether satisfactory answer to this problem. As hardness decreases, the water may tend to become more corrosive. A polyelectrolyte is therefore a very desirable, though optional, component of the cleaning solutions.

Polyelectrolytes are high molecular weight electrolytes; and they are either of natural origin, such as proteins, or they are of a synthetic nature, such as polymerized organic acids. Since the polyelectrolytes in solution do not dissociate to give a uniform distribution of positive and negative ions, as do simple electrolytes, the ions of one sign are bound to the polymer chain. Thus, for instance, the negative charges may be in the polymer chain, and only positive ions will be free to diffuse through the solvent.

The polyelectrolytes used in the solutions used in this invention can be any of the compounds known to prevent precipitation of the minerals which cause water-hardness, but certain preferences can usefully be borne in mind. Because phosphates may be regarded as environmentally-objectionable, we prefer to use a polyelectrolyte which does not contain phosphates, since then the plant effluent will not contain phosphates. We also prefer to avoid the use of the previously employed alkali metal tripolyphosphates, because these may have the deleterious effect of promoting etching or de-tinning. Because they do not promote de-tinning and possibly may to some extent inhibit etching the polyelectrolytes which we prefer for use in the cleaning solutions are polyelectrolytes such as Gantrez S-95 ("Gantrez" is a trade mark), manufactured by GAF Corporation, and Tamol 960 ("Tamol" is a trade mark) manufactured by Rohm and Haas Company.

The polyelectrolytes will preferably be present in a concentration which is effective substantially to prevent precipitation of the calcium and magnesium ions that are the primary cause of water-hardness. Generally, the greater the hardness of the water the greater will be the desired concentration of the polyelectrolyte. We have found that the concentration of polyelectrolyte will preferably be at least about 0.1 g/I, and most advantageously in the range of from about 0.1 g/I to about 1 g/I. There is no objection to the use of concentrations in excess of 1 /gl, but in our experience such higher concentrations do not result in any significant improvement.

One or more surfactants or wetting agents can usefully be added to the aqueous alkaline cleaning solutions used in the present invention, so as to enhance the performance of the cleaning solution in a conventional manner-but the presence or absence of surfactants has no noticeable effect as regards either inhibiting or promoting the etching of the tin surface by the cleaning solution. Supposing a surfactant is added which is not a low-foaming surfactant, then a defoaming agent will also desirably be added-since otherwise foaming can become so serious as to cause delay or even shut-down in a commercial cleaning line.

The surfactants and wetting agents employed in the cleaning solutions can for instance be ethoxylated straight-chain alcohols and octyl or nonyl phenoxy polyethoxyethanol. Nonionic surfactants are usually preferred since they are low-foaming.

The cleaning solutions will preferably contain at least about 0.2 g/I of the surfactant(s); particularly preferred concentrations are in the range of from about 0.2 g/I to about 0.5 g/I.

As already indicated, the cleaning solution must have a pH value (determined at a solution temperature of about 27°C) within the range of from about 11 to about 13; and will preferably have a pH value within the range of from about 12 to about 12.8.

The alkaline component used in the cleaning solution used in the process of this invention may be of any kind known to produce an alkaline solution when dissolved in water; but it will preferably not be an environmentally-objectionable one. The alkaline component therefore can advantageously be one or a mixture of more than one alkali metal hydroxides and/or carbonates and/or silicates and/or ammonium hydroxides and/or carbonates. A particlarly preferred alkaline component is a mixture of sodium carbonate, sodium metasilicate and either sodium hydroxide or potassium hydroxide or both.

The alkaline component must naturally be present in a concentration which will be effective substantially to remove lubricants or other such soiling contaminants. The minimum effective amount may be readily determined in the conventional manner. The concentration of alkaline component in the solution will preferably be at least about 2 g/I, and more advantageously will be in the range of from about 3 g/I to about 5 g/I. Greater concentrations may be employed, but the benefit to be gained thereby is generally not significant.

Tin surfaces may be cleaned by contacting them with the aqueous alkaline cleaning solutions for a sufficient time at the chosen temperature to remove lubricants or other such soiling contaminants therefrom, without visibly etching the tin surface. Usually the solution temperature should be at least about 100°F (38°C); and it will preferably be in the range of from about 100°F to about 130°F (38° to 54°C) and above all from about 115°F to about 125°F (46° to 52°C). The optimum temperature may tend to be somewhat higher for solutions with low concentrations of alkaline components than for solutions with higher concentrations thereof-or, put another way, the optimum treatment temperature tends somewhat to vary inversely with the pH of the cleaning solution.

The necessary period of treatment will generally depend on the method of application. Spraying is the preferred method, and when used the treatment time will tend to decrease as the spraying pressure increases. Operating at currently conventional spraying pressures of about 25 psig (pounds per square inch, gauge pressure) to about 35 psig (1.76 to 2.46 kg/cm²) it should be found that treatment times of from about 40 seconds up to about one minute may be sufficient to produce a water-break-free surface. If one employs the already-known but little used spraying pressures of 60 psig to 100 psig (4.22 to 7.03 kg/cm²) then the treatment times may be reduced, perhaps to as little as from about 1 to 5 seconds.

The treatment time may need to be increased the longer the interval between manufacture of the tin-plated metal article and the cleaning thereof. With drawn-and-ironed tin-plated steel cans, an interval between manufacture and cleaning of as little as fifteen minutes may necessitate a noticeably increased cleaning time. The necessary treatment time may also vary depending on the type of lubricant used in the manufacturing process; some being more readily removed than others.

In order to discover the extent to which the cleaning solutions will inhibit etching we have used treatment times of up to about 30 minutes without visibly etching the tin; bit in actual practice is it of course recommended to use the shortest treatment time which is effective to produce a water-break-free surface without etching the tin.

After the tin surface has been cleaned with the cleaning solution, the clean surface will generally be rinsed at least once with tap water, and then may advantageously be rinsed with deionized water and dried at an elevated temperature, preferably one in the range of from about 350° to about 400°F (177°to250°C).

It is convenient to make up the cleaning solutions from either an aqueous concentrate or a solid cleaning composition, which can simply be added to water to produce the desired aqueous alkaline cleaning solutions.

Such an aqueous concentrate may advantageously be formulated so that when added to water at a concentration in the range of from about 0.5% to about 2% by volume, and preferably in the range of from about 1% to about 2% by volume, it produces an aqueous alkaline cleaning solution having a pH of about 11 to about 13, and comprises an alkaline component in an amount effective substantially to remove contaminants from the tin surface, as well as one of the herein-defined inhibitors in an amount effective to inhibit etching of the surface. The alkaline component will preferably constitute up to about 770 grams per litre, and advantageously from about 250 to about 500 grams per litre of the concentrate. The inhibitor will preferably constitute at least about 2 grams per litre, and advantageously from about 2 to about 6 grams per litre of the concentrate. The concentrate optionally but desirably will also contain polyelectrolyte(s) and/or surfactant(s). The polyelectrolyte will desirably be present in a concentration within the range of from about 10 to about 20 grams per litre.

Alternatively a solid cleaning composition may advantageously be formulated so that when added to water at a concentration of from about 3 g/I to about 7 g/I, and preferably from about 4.6 g/I to 6.7 g/I, it will produce an aqueous alkaline cleaning solution having a pH of about 11 to about 13 and contains an effective amount of an alkaline component and an effective amount of an inhibitor as defined above. The alkaline component will preferably constitute at least about 15% by weight of the composition. The inhibitor will preferably constitute at least about 0.1% by weight, and most advantageously from about 0.5% to about 2% by weight of the composition. Moreover the composition optionally but desirably will also contain a polyelectrolyte, present preferably in a concentration of up to about 10% by weight, and most advantageously in a concentration of from about 3% to about 10% by weight of the composition.

The balance (if any) of the cleaning composition may consist of diluents and the like, that is to say compounds which can be regarded as inert with respect to any possible influence, either positive or negative, upon the cleaning and non-etching properties of the cleaning solutions of the invention. A typical but merely illustrative example of such compounds is for instance sodium sulphate.

In order that the invention may be well understood, it will now be described in more detail, but only by way of illustration, in the following examples:
Examples

It should first be noted that, in each of the following Examples, sets of "drawn-and-ironed" tin-plated steel cans (previously defined and hereinafter called Di cans) were contacted with the specified cleaning solution within 24 hours of their manufacture, and without any other treatment prior to contact with the cleaning solutions of the invention.

The cleaning solutions were made up from solid cleaning compositions having the components indicated in Table I below present in the percentages there shown. Each such composition is identified in Table I and elsewhere by a number and the subscript "c". The solutions were made up by dissolving a specific amount, in grams, of each composition as indicated in Table II below to 6 litres of water, to form aqueous alkaline cleaning solutions having the concentrations of components (including surfactants) indicated in Table III below. Each such cleaning solution is identified in Table III and elsewhere by the number of the composition from which it has been made, coupled with the subscript "s".

In each of the Examples the sets of cans were contacted with the cleaning solution by spraying them with the solutions at about 25 psi (1.76 kg/cm²) for the periods and at the temperatures there stated; and afterwards the cans were then rinsed with water, and visually examined for etching and appearance.

### Example 1

A set of DI cans was sprayed with cleaning solution 1s for 10 minutes at 123°F (about 51 °C). The results obtained are summarized in Table IV as follows:

### Example 2

Sets of DI cans were sprayed with cleaning solutions 2s, 3s and 4s, one set per test, for the times and at the temperatures indicated; and the results observed are summarized in Table V as follows:

### Example 3

Cleaning solutions 5s, 6s and 7s were prepared using tap water, and having the concentrations of components indicated in Table VI below. Solution 7s does not contain an inhibitor, and thus (like cleaning solution 1 s in Example 1) is presented only for purposes of comparison.

Sets of Di cans were sprayed with cleaning solutions 5s, 6s and 7s, one set per test, at solution :emperatures of 124°F (α51°C) for the times indicated; and the results obtained are summarized in Table VII as follows:

## Claims

1. A process for removing lubricants or other soiling contaminants from a tin surface without visibly etching it, in which the surface is brought into contact for a sufficient time at the chosen temperature with an aqueous alkaline cleaning solution having a pH in the range of from 11 to 13 and containing effective amounts of an alkaline component and of an inhibitor, characterized in that inhibitor is or includes one or more substituted or unsubstituted quinones and/or substituted or unsubstituted dihydroxybenzenes, the or each substituent on the quinone or dihydroxybenzene being hydroxy, halo, alkyl, alkoxy, nitro or cyano.

2. A process according to claim 1 characterized in that the inhibitor is or includes a substituted or unsubstituted quinone conforming to one of the general formulae in which R1_{'} R₂, R₃ and R₄ are the same or different and each represents a hydrogen atom or a hydroxy, halo, alkoxy, alkyl, nitro or cyano group.

3. A process according to claim 2 characterized in that the inhibitor is or includes 1,4-benzoquinone and/or 1,2-benzoquinone.

4. A process according to claim 1 characterized in that the inhibitor is or includes the substituted or unsubstituted dihydroxybenzene, and the substituted or unsubstituted dihydroxybenzene is substituted or unsubstituted ortho-dihydroxybenene.

5. A process according to claim 1 characterized in that the inhibitor is or includes one or more of the following, namely resorcinol (meta-dihydroxybenzene), hydroquinone (1,4-dihydrobenzoquinone or para-dihydroxybenzene) and 1,3,5-trihydroxybenzene.

6. A process according to claim 1 characterized in that the inhibitor is or includes one or more of the following, namely catechol (ortho-dihydroxybenzene), hydroxy-hydroquinone (1,2,4-trihydroxybenzene) and 1,2,4,5-tetrahydroxybenzene.

7. A process according to any one of the preceding claims characterized in that the inhibitor is present in a concentration in the range of from 0.02 g/I to 0.06 g/I.

8. A process according to any one of the preceding claims characterized in that the solution includes a polyelectrolyte in a concentration effective substantially to prevent precipitation.

9. A process according to claim 8 characterized in that the polyelectrolyte is present in a concentration of at least 0.1 g/I.

10. A process according to any one of the preceding claims characterized in that the temperature employed is in the range of from 38° to 54°C.

11. A process according to any one of the preceding claims characterized in that it includes the preliminary step of making-up the aqueous alkaline cleaning solution by dissolving from 3 g/I to 7 g/I of a solid cleaning composition in water, at least 15% by weight of the composition being formed by the alkaline component and at least 0.1 % by weight of the composition being formed by the inhibitor, said composition also optionally including a polyelectrolyte in a proportion effective substantially to prevent precipitation of calcium and magnesium ions in hard water.

12. A process according to any one of claims 1-10 characterized in that it includes the preliminary step of making-up the aqueous alkaline cleaning solution by dissolving from 0.5% to 2% by volume of an aqueous concentrate in water, said concentrate containing up to 770 g/I of the alkaline component and at least 2 g/I of the inhibitor, as well as optionally a polyelectrolyte in a proportion effective substantially to prevent precipitation of calcium and magnesium ions in hard water.

## Patentansprüche

1. Verfahren zur Entfernung von Schmiermitteln oder anderen verschmutzenden Verunreinigungen von einer Zinnoberfläche ohne diese sichtbar zu ätzen, wobei die Oberfläche in Berührung gebracht wird während einer ausreichenden Zeit bei einer gegebenen Temperatur mit einer wässrigen alkalischen Reinigungslösung, die einen pH-Wert im Bereich von 11 bis 13 aufweist und wirksame Mengen einer alkalischen Komponente und eines Inhibitors enthält, dadurch gekennzeichnet, daß der Inhibitor aus einem oder mehreren substituierten oder unsubstituierten Chinonen und/oder substituierten oder unsubstituierten Dihydroxybenzolen besteht oder solche enthält, wobei die Substituentten an dem Chinon oder Dihydroxybenzol Hydroxy, Halogen, Alkyl, Alkoxy, Nitro oder Zyano sein können.

2. Verfahren gemäß Anspruch 1, dadurch gekennzeichnet, daß der Inhibitor ein substituiertes oder unsubstituiertes Chinon entsprechend der allgemeinen Formel enthält oder aus einem solchen besteht, wobei in den allgemeinen Formeln R_{1'} R_{2'} R₃ und R₄ gleich oder verschieden sein können und jeweils ein Wasserstoffatom oder eine Hydroxygruppe, Halogen, Alkoxygruppe, Alkylgruppe, Nitrogruppe oder Zyanogruppe bedeuten.

3. Verfahren gemäß Anspruch 2 dadurch gekennzeichnet, daß der Inhibitor 1,4-Benzochinon und/oder 1,2-Benzochinon ist oder solches enthält.

4. Verfahren gemäß Anspruch 1, dadurch gekennzeichnet, daß der Inhibitor aus einem substituierten oder unsubstituierten Dihydroxybenzol besteht oder solches enthält, wobei das substituierte oder unsubstituierte Dihydroxybenzol substituiertes oder unsubstituiertes Ortho-Dihydroxybenzol ist.

5. Verfahren gemäß Anspruch 1, dadurch gekennzeichnet, daß der Inhibitor aus einer oder mehreren der folgenden Verbindungen besteht oder solche enthält: Resorcin(meta-Dihydroxybenzol), Hydrochinon (1,4-Dihydrobenzochinon oder para-Dihydroxybenzol) und 1,3,5-Trihydroxybenzol.

6. Verfahren gemäß Anspruch 1, dadurch gekennzeichnet, daß der Inhibitor aus einer oder mehreren der folgenden Verbindungen besteht oder solche enthält: Katechol (ortho-Dihydroxybenzol), Hydroxy-Hydrochinon (1,2,4-Trihydroxybenzol) und 1,2,4,5-Tetrahydroxybenzol.

7. Verfahren gemäß einem der vorgehenden Ansprüche dadurch gekennzeichnet, daß der Inhibitor anwesend ist in einer Konzentration im Bereich von 0,02 g/I bis 0,06 g/I.

8. Verfahren gemäß einem der vorgehenden Ansprüche, dadurch gekennzeichnet, daß die Lösung einen Polyelektrolyt enthält in einer Konzentration die im wesentlichen wirksam ist um eine Ausfällung zu vermeiden.

9. Verfahren gemäß Anspruch 8, dadurch gekennzeichnet, daß der Polyelektrolyt anwesend ist in einer Konzentration von mindestens 0,1 g/I.

10. Verfahren gemäß einem der vorgehenden Ansprüche, dadurch gekennzeichnet, daß die angewandte Temperatur im Bereich von 38 bis 54°C liegt.

11. Verfahren gemäß einem der vorgehenden Ansprüche, dadurch gekennzeichnet, daß es einschließt die Vorstufe der Herstellung der wässrigen alkalischen Reinigungslösung durch Auflösen von 3 g/I bis 7 /gl einer festen Reinigungszusammensetzung in Wasser, wobei mindestens 15 Gew.-% der Zusammensetzung von der alkalischen Komponente gebildet werden und mindestens 0,1 Gew.-% der Zusammensetzung von dem Inhibitor gebildet werden, und wobei die Zusammensetzung auch gegebenenfalls einen Polyelektrolyten enthält in einer Menge, die im wesentlichen wirksam ist um eine Ausfällung von Kalzium- und Magnesiumionen in hartem Wasser zu vermeiden.

12. Verfahren gemäß einem der Ansprüche 1 bis 10, dadurch gekennzeichnet, daß es einschließt die Vorstufe der Herstellung der wässrigen alkalischen Reinigungslösung durch Auflösen von 0,5 bis 2 Vol.-% eines wässrigen Konzentrats in Wasser, wobei dieses Konzentrat bis zu 770 g/I der alkalischen Komponente und mindestens 2 g/I des Inhibitors enthält, sowie gegebenenfalls einen Polyelektrolyten in einer Menge, die im wesentlichen wirksam ist, um eine Ausfällung von Kalzium- und Magnesiumionen in hartem Wasser zu verhindern.

## Revendications

1. Un procédé d'élimination de lubrifiants ou d'autres contaminants salissants à partir d'une surface d'étain sans la rayer visiblement, dans lequel la surface est mise en contact pendant un temps suffisant, à la température choisie avec une solution de nettoyage alcaline aqueuse ayant un pH dans le domaine de 11 à 13 et contenant des quantités efficaces d'un composant alcalin et d'un inhibiteur, caractérisé en ce que l'inhibiteur est ou inclut une ou plusieurs quinones substituées ou non substituées et/ou dihydroxybenzènes substitués ou non substitués, le substituant ou chacun des substituants sur la quinone ou le dihydroxybenzène étant un groupe hydroxy, halogène, alcoyle, alcoxy, nitro ou cyano.

2. Un procédé selon la revendication 1, caractérisé en ce que l'inhibiteur est ou inclut une quinone substituée ou non substituée conformement à celles de formule générale: dans laquelle R,, R₂, R₃ et R₄ sont identiques ou différents et représentent chacun un atome d'hydrogène ou un groupe hydroxy, halogène, alcoxy, alcoyle, nitro ou cyano.

3. Un procédé selon la revendication 2, caractérisé en ce que l'inhibiteur est ou inclut la 1,4-benzoquinone et/ou la 1,2-benzoquinone.

4. Un procédé selon la revendication 1, caractérisé en ce que l'inhibiteur est ou inclut le dihydroxybenzène substitué ou non substitué et en ce que le dihydroxybenzène substitué ou non substitué est de l'ortho-dihydroxybenzène substitué ou non substitué.

5. Un procédé selon la revendication 1, caractérisé en ce que l'inhibiteur est ou inclut un ou plusieurs des composés suivants, à savoie le résorcinol (méta-dihydroxybenzène), l'hydroquinone (la, 1,4-dihydroxybenzoquinone ou le para-dihydroxybenzène) et le 1,3,5-trihydroxybenzène.

6. Un procédé selon la revendication 1, caractérisé en ce que l'inhibiteur est ou inclut un ou plusieurs des composés suivants, à savoir le catéchol (ortho-dihydroxybenzène), l'hydroxy-hydroquinone (1,2,4-trihydroxybenzène) et le 1,2,4,5-tétrahydroxybenzène.

7. Un procédé selon l'une quelconque des revendications précédentes, caractérisé en ce que l'inhibiteur est présent en une concentration dans le domaine de 0,02 g à 0,06 g/I.

8. Un procédé selon l'une quelconque des revendications précédentes, caractérisé en ce que la solution comprend un polyélectrolyte en concentration suffisamment efficace pour empêcher la précipitation.

9. Un procédé selon la revendication 8, caractérisé en ce que le polyélectrolyte est présent en une concentration d'au moins 0,1 g/I.

10. Un procédé selon l'une quelconque des revendications précédentes, caractérisé en ce que la température utilisée est dans le domaine de 38 à 54°C.

11. Un procédé selon l'une quelconque des revendications précédentes, caractérisé en ce qu'il comprend l'étape préliminaire de fabrication de la solution de nettoyage alcaline aqueuse en dissolvant de 3 g/I à 7 g/I d'une composition solide de nettoyage dans l'eau, au moins 15 % en poids de la composition étant formés par le composant alcalin et au moins 0,1 % en poids de la composition étant formé par l'inhibiteur, ladite composition comprenant aussi éventuellement un polyélectrolyte en proportions suffisamment efficaces pour éviter la précipitation d'ions calcium et magnésium dans l'eau dure.

12. Un procédé selon l'une quelconque des revendications 1 à 10, caractérisé en ce qu'il comprend l'étape préliminaire de fabrication de la solution de nettoyage alcaline aqueuse en dissolvant de 0,5 à 2 % en volume d'un concentrat aqueux dans l'eau, ledit concentrat contenant jusqu'à 770 g/I de composant alcalin et au moins 2 g/I d'inhibiteur ainsi qu'éventuellement un polyélectrolyte dans une proportion suffisamment efficace pour empêcher la précipitation d'ions calcium et magnésium dans l'eau dure.
